

Dec. 12, 1972

R. G. GRIGOROVICI ET AL  
PIEZORESISTIVE TRANSDUCERS AND DEVICES WITH SEMICONDUCTING  
FILMS AND THEIR MANUFACTURING PROCESS  
Filed July 14, 1971

3,705,993



Fig.1



Fig. 2



Fig. 3

Radu GRIGOROVICI et al.  
Inventors

Karl F. Ross

Attorney



torr. Thereafter the previously degased germanium is deposited by evaporation from the tungsten wire onto the mica substrate maintained at a temperature between 470° and 500° C., with a deposition rate less than 2,000 A./minute to form the polycrystalline film 3.

After removing the substrate from the furnace, silver wire terminals 5 are fastened by gummed transparent tape 4 onto the substrate in the inactive region in such a way, that an electric contact between the electrodes and the terminals may be made by soldering with colloidal-silver paste 6. The whole surface of mica substrate is covered on that side on which the piezoresistive element is deposited, with a protecting lacquer 7. Thereafter, the element thus obtained is cut along the outline of the mica substrate and the piezoresistive devices are then sorted and calibrated.

When kapton substrates are used, the operations are identical to those with mica substrates, with the only difference being the deposition temperature of the polycrystalline germanium. During the deposition operation the substrate is maintained at a temperature of 300°-375° C.

#### Example 2

On a metallic substrate 8 (FIG. 3) of carbon steel of at least 0.1 mm. thickness, degreased and etched by a detergent and sulphuric acid or hydrochloric acid, thereafter neutralized with sodium carbonate, borax and sodium nitrate and dried, a heat-resistant enamel film 9 of max. 0.4 mm. thickness is applied by pouring, simple spraying, by spraying in an electrostatic field, or by electrophoresis. After air-drying at up to 120° C., the substrate is placed in a furnace previously heated at 800-830° C., for 3-4 minutes, in the burning in zone. On the side of the substrate opposite that on which the transducer is to be deposited and which may come into contact with a corroding medium, the surface may be protected either by means of a stainless steel film 10, or a heat-resistant acid- and alkali-proof enamel layer. The thus prepared substrate is placed with its side opposite to that on which the transducer is to be deposited on a copper furnace surface to bond colloidal-silver paste strips thereto as described. After the paste is dried the electrodes 11 are painted by means of a pattern with colloidal-silver paste or a paste of gold solution. Thereafter the inactive surfaces are masked with 20-microns-thick aluminum foil strips, the outer halves of the electrodes being similarly masked. On each electrode there are deposited according to requirements several transducers 12.

A filament is made from 0.2-0.5 mm. diameter plaited wires, in to the meshes of which are fastened by pressing small pieces of polycrystalline germanium. The substrate is degased at 470°-550° C. over a period of 30-60 minutes, in vacuum, at a pressure  $p < 5 \times 10^{-5}$  torr. After that, the previously degased germanium is deposited by evaporation in vacuum on the enamel-covered metallic substrate, the temperature of the substrate during the deposition being between 470° and 530° C., the deposition rate being less than 2,000 A./minute.

After the substrate with the deposited transducer is removed, the terminals 13 out of 0.1 mm. diameter silver wire are fastened on the uncovered side of the electrodes by means of silver paste, after which the whole transducer element is covered by a heat-resistant lacquer 14.

#### Example 3

According to Example 2, a maximum 0.1 mm. thick enamel film is applied on the surfaces of steel parallel-pipeds of different sizes, as for instance 10 x 10 x 15 mm. On the enamel, employing a convenient pattern, are deposited an electrode of a gold solution by painting and thermal treatment at 700° C., during 5 minutes. The specimen thus obtained is correspondingly masked for instance by means of aluminum foil and is introduced into a small tantalum boat of adequate dimensions, with

which the specimen is heated in vacuum to 350°-400° C. at a pressure  $p < 5 \times 10^{-5}$  torr. On the thus-prepared support is deposited the polycrystalline Ge film, as in Example 2. Thereafter the contacts are laid and the device is covered with heat-resistant lacquer, as in Example 2.

The thus-obtained device can be utilized for measuring stresses, signalling limit stresses, and for other tensiometrical measurements.

This invention offers the advantages of a gauge factor  $G=30$ , a linear variation of  $dR/R$  with  $\delta$ , as well as a temperature coefficient of the gauge factor and of the electric resistance of say  $-1 \times 10^{-3}$  to  $-5 \times 10^{-4}$ /degree C. in each case. The device also has a good time constancy, as well for R as for G; the stability of R is better than  $\pm 0.2\%$  in 24 hours at 20° C. and that of G better than  $\pm 0.05\%$  in 24 hours at 20° C. In addition better adherence is ensured between the polycrystalline film and the substrate, allowing measurements at large mechanical deformations, the maximum admissible deformation being  $1 \times 10^{-3}$ ; the deviation from linearity at a maximum deformation  $\delta$  between  $6 \times 10^{-4}$  and  $10 \times 10^{-4}$  being beneath 0.2%. The device utilizes as raw material polycrystalline germanium, which is much cheaper than the single crystals, allows the formation of well fastened terminals, which ensure a perfect electric contact and ruggedness, is protected against external agents, and ensures a more secure fastening of the transducer on the article whose deformation is to be measured in such way, that it forms practically a single body therewith. We are able to obtain an insulating film adherent to carbon steel, stainless steel or steel platings, without pin-holes, heat-resistant, and to use the device in corroding media.

We claim:

1. A method of making a piezoresistive mechanical-electrical transducer, comprising the steps of:  
applying to a heat-resistant substrate at least two conductive strips in spaced-apart relationship;  
vacuum-evaporating onto said substrate over a limited region thereof bridging said strips, polycrystalline germanium at a temperature between substantially 330° C. and 600° C. at a pressure less than substantially  $5 \times 10^{-5}$  torr at a rate up to about 2000 A./per minute to form a germanium layer;  
soldering wire terminals to said strips; and  
coating said substrate and said strips and the germanium layer with a layer of a heat-resistant lacquer.
2. The method defined in claim 1 wherein said substrate is selected from the group which consists of mica, kapton or enamel-coated metal, said strips are applied to said substrate at room temperature and said wires are bonded to said substrate by epoxy resin.
3. The method defined in claim 2 wherein said substrate is composed of steel coated with an enamel to a maximum thickness of 0.4 mm. and is fired at a temperature between substantially 800° C. and 900° C. for a period of 3 to 4 minutes.
4. The method defined in claim 1 wherein said strips consist of silver, gold or platinum paste fired to bond the strips to the substrate or are constituted of silver, platinum, aluminum, gold, nickel or molybdenum film.
5. The method defined in claim 4 wherein said strips are formed by applying colloidal-silver conductive paste to said substrate and heating said substrate with the colloidal-silver conductive paste thereon to form the strips and simultaneously bond the same to said substrate.
6. A piezoresistive mechanical-electrical transducer comprising:  
a substrate selected from the group which consists of mica, capton or iron coated with enamel and baked at substantially 800° C. to 900° C. for a period of 3 to 4 minutes;  
two spaced-apart conductive strips selected from the group which consist of silver, gold, platinum, aluminum, nickel or molybdenum on said substrate;

- a polycrystalline germanium layer extending over a limited region of said substrate and bridging said strips;
- a wire terminal soldered to each of said strips and bonded by epoxy resin to said substrate; and
- a layer of heat-resistant lacquer coating said substrate, said strips and said layer.

- |           |        |                      |           |
|-----------|--------|----------------------|-----------|
| 3,505,572 | 4/1970 | Yamashita et al. --- | 310—8.1 X |
| 3,585,415 | 6/1971 | Muller et al. -----  | 310—8     |
| 3,460,005 | 8/1969 | Kandu et al. -----   | 310—8 UX  |

## FOREIGN PATENTS

- |   |         |        |               |         |
|---|---------|--------|---------------|---------|
| 5 | 517,928 | 8/1953 | Belgium ----- | 310—9.7 |
|---|---------|--------|---------------|---------|

JOSEPH V. TRUHE, Primary Examiner

B. A. REYNOLDS, Assistant Examiner

10

U.S. CL. X.R.

29—25.35, 594; 73—88.5; 310—8.5; 338—5

## References Cited

## UNITED STATES PATENTS

- |           |         |                        |           |
|-----------|---------|------------------------|-----------|
| 3,137,834 | 6/1964  | Pfann -----            | 73—88.5 X |
| 3,290,569 | 12/1966 | Weimer -----           | 307—308 X |
| 3,492,513 | 1/1970  | Hollander et al. ----- | 338—2 X   |